

## UNITED STATES PATENT OFFICE

1,988,803

PROCESS FOR THE PRODUCTION OF  
LUBRICATING OILDavid R. Merrill, Long Beach, Calif., assignor to  
Union Oil Company of California, Los Angeles,  
Calif., a corporation of CaliforniaNo Drawing. Application October 30, 1933  
Serial No. 695,957

11 Claims. (Cl. 196—13)

This invention relates to a process for the treatment of petroleum. More specifically it relates to a process for the treatment of petroleum with selective solvents.

5 In the production of lubricating oil for internal combustion motors it is highly desirable to obtain a product which exhibits a low temperature viscosity susceptibility, a low Conradson carbon value, a high stability towards sunlight and a low 10 oxidation value. Crude lubricating oil fractions produced either as distillates or as residues are usually composed of mixtures of paraffinic, naphthenic, aromatic and olefinic hydrocarbons. The olefinic hydrocarbons are highly unsaturated and 15 their presence in the finished lubricating oil is undesirable because of their unstable characteristics. These compounds are unstable and usually darken when exposed to sunlight. Furthermore, they have a high tendency towards polymerization with the result, after a considerable 20 period, that these compounds are converted into resinous substances which increase the sludge value of the oil.

The aromatic and naphthenic hydrocarbons 25 present in crude lubricating oil fractions are undesirable because of their high temperature viscosity susceptibility. These compounds exhibit too great a change in viscosity for a given change in temperature. The paraffinic hydrocarbons 30 present in crude lubricating oil fractions are the most desirable materials to be employed as lubricants. These compounds are highly saturated hence, from a chemical standpoint, they are rather inactive and do not exhibit a tendency towards 35 the formation of undesirable resinous or sludge forming constituents. Furthermore, these compounds exhibit a low temperature viscosity susceptibility. In other words, they exhibit a minimum change in viscosity for a given change in 40 temperature. Furthermore, these highly saturated hydrocarbons are relatively stable to sunlight, undergoing little change in color on exposure. When I use the term "paraffinic hydrocarbons" I mean those compounds which are present 45 in petroleum having the aforementioned characteristics and which are liquid at ordinary temperatures. This group of hydrocarbons does not include those compounds present which are usually solid or semi-solid at ordinary temperature and which are known as "wax" or "petrolatum".

In the production of lubricating oil from crude petroleum residues or distillates, it is becoming conventional in the art to separate the desirable 50 paraffinic hydrocarbons from the undesirable

olefinic, naphthenic and/or aromatic compounds by the use of solvents which selectively dissolve the undesirable hydrocarbons present in the petroleum fraction but which exhibit only a very limited solvent power on the desirable paraffinic hydrocarbons. 5

As a matter of convenience hereafter, I will refer to the desirable lubricating oil constituents of petroleum as the "paraffinic" hydrocarbons and to the undesirable constituents, such as olefinic, naphthenic and/or aromatic hydrocarbons as the "non-paraffinic" constituents of petroleum. 10

A number of selective solvents have been found desirable to separate the paraffinic from the non-paraffinic hydrocarbons, for example, it has been 15 shown that such materials as sulphur dioxide, beta beta dichlorethyl ether, chloraniline, nitrobenzene, aniline and furfural are highly selective as solvents for the non-paraffinic hydrocarbons. The foregoing selective solvents are relatively 20 heavy as compared to petroleum. When these relatively heavy solvents are commingled with petroleum or petroleum fractions under the proper conditions of temperature, the undesirable 25 non-paraffinic hydrocarbons present pass into solution to a greater or less extent but the desirable paraffinic hydrocarbons remain largely undissolved. If the commingled mass is allowed to remain in a quiescent state the solution of undesirable hydrocarbons settles to the bottom of the 30 container and forms what is known as an "extract" phase. The relatively light paraffinic hydrocarbons rise to the top of the vessel and form a raffinate phase. These phases are then readily 35 separable by ordinary decantation means. The raffinate phase is usually found to contain a small quantity of the selective solvent and the extract phase ordinarily contains a relatively large quantity of the solvent. These fractions 40 may be purified by subjecting them to distillation 45 whereby the solvent is distilled away from the hydrocarbon oils.

The conventional method of separating the undesirable non-paraffinic hydrocarbons from a hydrocarbon mixture consists in treating this 45 mixture with a selective solvent under the proper conditions of temperature by the addition of sufficient solvent to the oil to remove the major portion of these undesirable hydrocarbons. Where one portion of the selective solvent is insufficient 50 to remove the major portion of the undesirable hydrocarbon present the method of treatment may be modified and the oil may be successively treated several times by the addition of fresh solvent to the partially treated oil until a highly 55

refined oil is obtained which is relatively free from the undesirable hydrocarbons. For example, an oil may be treated with liquid sulphur dioxide at a temperature of about 10° F. and the raffinate so obtained may be successively treated with sulphur dioxide at the same temperature until the major portion of non-paraffinic hydrocarbons have been extracted from the oil. The major portion of the undesirable hydrocarbons are usually removed by the first treatment with the selective solvent and the remaining undesirable hydrocarbons are then removed to a greater or less extent by the successive treatments.

It has also been proposed to regulate the solvent power of the extracting agent at any stage of the treatment in accordance with the solubility of the material to be extracted and as the refining of the stock by extraction progresses in a step-wise manner the solvent power of the treating agent should be increased.

By substantially increasing the solvent power or ease of miscibility of the treating agent, it is possible to fractionate the raffinate, obtained after extraction with the pure solvent, into a further extract of lower solubility than the first extract obtained by the use of said pure solvent and a second raffinate of consequently still lower solubility than the first raffinate.

It has been found desirable to first extract a hydrocarbon mixture with a pure selective solvent, such as aniline, nitrobenzol, sulphur dioxide, furfural, dichlorethyl ether or chloraniline and then re-treat the raffinate so produced with a modified solvent, or with the same solvent at a higher temperature. As modifying agents such materials as carbon bisulphide, xylene, benzene, toluene, carbon tetrachloride, ethers or tetrachlorethane, may be employed.

By these processes the oil feed is divided in one general operation into three or more fractions of different viscosity-gravity constants.

The viscosity-gravity constant referred to in this application has been determined by the method employed by Hill and Coates set forth in the Journal of Industrial and Engineering Chemistry, Vol. 20, page 641 of 1928. This constant represents the paraffinicity or naphthenicity of an oil. A high value represents a high degree of naphthenicity while low values indicate relatively greater paraffinicity. Lubricating oils from natural crudes range from 0.903 viscosity-gravity constant for an extreme Gulf Coast type to 0.807 for an extreme Pennsylvania type, or even beyond.

For example, in a two stage extraction of lubricating oil using selective solvents, the first stage results in a primary raffinate and a low quality extract. To produce a high quality raffinate from the primary raffinate, the latter is again extracted, with the same or a different selective solvent than that first employed. As previously stated, this second extraction may be in the presence of a modifying agent described above. Another raffinate and extract are produced from the primary raffinate, resulting in a high quality raffinate and an intermediate grade extract. The high quality raffinate can be further purified, if desired, by further successive extractions and each of these successive extractions results in an intermediate grade extract.

I have found that in a solvent extraction process involving these successive extractions some of the lighter, less viscous lubricating oils having low viscosity-gravity constants are present in the intermediate grade extract rather than in the

high quality raffinate as desired. I believe that these valuable fractions are present in the intermediate extract's instead of in the high quality raffinate because the oils of lower molecular weight or lower viscosity tend to be somewhat more soluble than fractions of higher molecular weight or higher viscosities having the same viscosity-gravity constant. The loss of high grade fractions in the intermediate grade extracts is undesirable.

It is an object of my invention to conserve the high grade fractions in the raffinate produced by extracting mineral oils by selective solvents.

It is a further object of my invention to extract a hydrocarbon mixture with a selective solvent and thereafter re-extract the raffinate so produced with a selective solvent which may or may not contain a modifying agent, and to recover from the intermediate grade extracts the valuable lighter, less viscous lubricating oils having desira- 20 ble low viscosity-gravity constants.

I have found that these objects may be accomplished by subjecting the intermediate grade extract to distillation so as to divide it into fractions of varying viscosity. The lighter fractions which are vaporized and separately condensed comprise the valuable, less viscous lubricating oils of low viscosity-gravity constants which would otherwise be lost in the intermediate extract.

On fractionation of the intermediate grade extract by distillation, the lower viscosity-gravity constant for the lighter fractions is ordinarily not so low that the light fractions may be mixed directly with the high grade raffinate although in some cases this may be done. I usually introduce the above mentioned recovered light fractions into the feed stage of a continuous countercurrent extractor wherein the selective solvent is introduced at an upper part of the extractor while the oil to be treated is introduced at a lower point. In some cases it is desirable to introduce said recovered light fractions above or below the point of introduction of fresh oil. This recovered material characterized by relatively low viscosity-gravity constant may be mingled with the primary raffinate for re-extraction in the presence of the selective solvent and the modifying agent.

As an example of my invention in operating on a feed stock having a wide range of molecular weights, I may use a de-asphaltized and dewaxed Kettleman Hills long residuum, having a gravity of 18.9° A. P. I. at 60° F., a Saybolt Universal viscosity of 97 seconds at 210° F., and a viscosity-gravity constant of 0.873. The dewaxed long residuum was extracted in countercurrent equipment with 200 volume percent. of sulphur dioxide at 115° F. and the raffinate so produced was then re-extracted in countercurrent equipment with 250 volume percent. of a mixture of 70% liquid sulphur dioxide and 30% benzene at 90° F. The raffinate produced by the re-extraction with the sulphur dioxide-benzene mixture had a gravity of 26.6° A. P. I. at 60° F., a Saybolt Universal viscosity of 86.5 seconds at 210 F., and a viscosity-gravity constant of 0.817. The intermediate extract produced by the SO<sub>2</sub>-benzene extraction having a gravity of 19.1° A. P. I., a Saybolt Universal viscosity of 102 seconds at 210° F., and a viscosity-gravity constant of 0.873 was then subjected to a fire and steam distillation and overhead fractions were obtained having the following characteristics:

Cut 1, gravity 26.7° A. P. I., Saybolt Universal 75

viscosity, 140 seconds at 100° F., and a viscosity-gravity constant of 0.849.

Cut 2, gravity 25.3° A. P. I., Saybolt Universal viscosity, 204.5 seconds at 100° F., and a viscosity-gravity constant of 0.853.

Cut 3, gravity 24.0° A. P. I., Saybolt Universal viscosity, 311 seconds at 100° F., and a viscosity-gravity constant of 0.857. The bottoms which remained after the removal of the three cuts

had the following characteristics:

Gravity 17.3° A. P. I., Saybolt Universal viscosity, 216 seconds at 210° F., and a viscosity-gravity constant of 0.875. The cuts were produced as aerial condensate and represented 7.1, 8.4, and

8.6% by volume of the intermediate extract.

On comparing the viscosity-gravity constants of the three cuts with the viscosity-gravity constant of the material before distillation and the bottoms from the distillation, it is evident that the cuts are of considerably lower viscosity-gravity constant, indicating the presence in them of appreciable proportions of high grade oil which preferably should be in the first grade oil raffinate rather than in intermediate grade extract.

In practice, therefore, the second grade oil such as the intermediate extract is subjected to distillation and a yield of distillate taken of approximately one-third of the charge to the still. This distillate is then condensed and returned to the extraction equipment either with the original feed or preferably with the feed to the second stage of operation, in which the raffinate from the first stage is extracted with the sulphur dioxide-benzene mixture. In this way these light fractions are subjected to a further extraction operation and the desirable constituents are to a considerable extent recovered in the form of first grade oil raffinate, thus increasing the yield of the latter material.

When no effort is made to recover the valuable products from the intermediate extract the yields in the foregoing example are as follows: high grade raffinate, 29.6%; intermediate grade extract, 45.4%; low grade extract produced by the primary extraction with liquid sulphur dioxide, 25.0%. However, when about one-third of the intermediate extract is vaporized, separately condensed and returned to the primary raffinate for reextraction with the liquid sulphur dioxide and benzol mixture, the yield of high grade raffinate may be increased from 29.6% to 34.3% with a corresponding reduction in the yield of intermediate grade extract.

It is to be understood that the foregoing is merely illustrative of one method of carrying out my invention and that many variations may be made by those skilled in the art within the scope of my invention which I claim:

60 I claim:

1. A process for the separation of paraffinic and non-paraffinic hydrocarbons from an oil containing the same which comprises extracting said oil in an extraction stage with a selective solvent, separating an extract fraction soluble in said selective solvent from a raffinate fraction insoluble therein, distilling said extract fraction to produce a light, viscous oil fraction having a lower viscosity gravity constant than the remaining extract fraction, and passing said distilled fraction to said extraction stage.

2. A process for the separation of paraffinic and non-paraffinic hydrocarbons from an oil containing the same which comprises extracting said oil in an extraction stage with a selective sol-

vent, separating an extract fraction soluble in said selective solvent from a raffinate fraction insoluble therein, distilling said extract fraction to produce a light, less viscous oil fraction having a lower viscosity gravity constant than the remaining extract fraction, passing said distilled fraction to said extraction zone and withdrawing a raffinate fraction from said extraction stage.

3. A process for the production of paraffinic and non-paraffinic hydrocarbons from oil containing the same which comprises extracting an oil in an extraction stage with a selective solvent and a modifying agent, separating an extract fraction soluble in said selective solvent and modifying agent from a raffinate fraction insoluble therein, distilling said extract fraction to produce a light, less viscous oil fraction having a lower viscosity gravity constant than the remaining extract fraction and passing said distilled fraction to said extraction stage.

4. A process as in claim 1 in which said extract fraction is fractionally distilled to produce said light, less viscous oil fraction.

5. A process for the separation of paraffinic and non-paraffinic hydrocarbons from a petroleum fraction containing the same which comprises extracting said oil with a selective solvent, separating the extracted fraction soluble in said selective solvent from the raffinate fraction insoluble therein, extracting said raffinate with a selective solvent to produce a high grade raffinate insoluble in said solvent and an intermediate grade extract soluble therein, separating said high grade raffinate from said intermediate grade extract, distilling light, less viscous lubricating oil having low viscosity gravity constant from said intermediate grade extract and mingling said light, less viscous lubricating oil with oil passing to the first mentioned extraction.

6. A process for the separation of paraffinic and non-paraffinic hydrocarbons from a petroleum fraction containing the same which comprises extracting said oil with a selective solvent, separating the extracted fraction soluble in said selective solvent from the raffinate fraction insoluble therein, extracting said raffinate with a selective solvent to produce a high grade raffinate insoluble in said solvent and an intermediate grade extract soluble therein, separating said high grade raffinate from said intermediate grade extract, distilling light, less viscous lubricating oil having low viscosity gravity constant from said intermediate grade extract and mingling said light, less viscous lubricating oil with oil passing to a previous extraction stage.

7. A process for the separation of paraffinic and non-paraffinic hydrocarbons from a petroleum fraction containing the same which comprises extracting said oil with a selective solvent, separating the extracted fraction soluble in said selective solvent from the raffinate fraction insoluble therein, extracting said raffinate with a selective solvent to produce a high grade raffinate insoluble in said solvent and an intermediate grade extract soluble therein, separating said high grade raffinate from said intermediate grade extract, distilling light, less viscous lubricating oil having low viscosity gravity constant from said intermediate grade extract and mingling said light, less viscous lubricating oil with said first mentioned raffinate for further extraction.

8. A process for the separation of paraffinic and non-paraffinic hydrocarbons from a petroleum fraction containing the same which com-

prises extracting said oil with a selective solvent, separating the extracted fraction soluble in said selective solvent from the raffinate fraction insoluble therein, extracting said raffinate with a selective solvent to produce a high grade raffinate insoluble in said solvent and an intermediate grade extract soluble therein, separating said high grade raffinate from said intermediate grade extract, fractionally distilling said intermediate grade extract to vaporize light, less viscous lubricating oil having low viscosity gravity constant, separately condensing said light, less viscous oil and mingling said light, less viscous lubricating oil with oil passing to the first mentioned extraction.

9. A process for the separation of paraffinic and non-paraffinic hydrocarbons from a petroleum fraction containing the same which comprises extracting said oil with a selective solvent, separating the extracted fraction soluble in said selective solvent from the raffinate fraction insoluble therein, extracting said raffinate with a selective solvent to produce a high grade raffinate insoluble in said solvent and an intermediate grade extract soluble therein, separating said high grade raffinate from said intermediate grade extract, fractionally distilling said intermediate grade extract to vaporize light, less viscous lubricating oil having low viscosity gravity constant, separately condensing said light, less viscous oil and mingling said light, less viscous lubricating oil with oil passing to a previous extraction stage.

10. A process for the separation of paraffinic and non-paraffinic hydrocarbons from a petroleum fraction containing the same which com-

prises extracting said oil with a selective solvent, separating the extracted fraction soluble in said selective solvent from the raffinate fraction insoluble therein, extracting said raffinate with a selective solvent and modifying agent to produce a high grade raffinate insoluble in said solvent and modifying agent and an intermediate grade extract soluble therein, separating said high grade raffinate from said intermediate grade extract, fractionally distilling said intermediate grade extract to vaporize light, less viscous lubricating oil having low viscosity gravity constant, separately condensing said light, less viscous oil and mingling said light, less viscous lubricating oil with oil passing to the first mentioned extraction.

11. A process for the separation of paraffinic and non-paraffinic hydrocarbons from a petroleum fraction containing the same which comprises extracting said oil with a selective solvent, separating the extracted fraction soluble in said selective solvent from the raffinate fraction insoluble therein, extracting said raffinate with a selective solvent and a modifying agent to produce a high grade raffinate insoluble in said solvent and modifying agent and an intermediate grade extract soluble therein, separating said high grade raffinate from said intermediate grade extract, fractionally distilling said intermediate grade extract to vaporize light, less viscous lubricating oil having low viscosity gravity constant, separately condensing said light, less viscous fraction and mingling said light, less viscous lubricating oil with oil passing to a previous extraction stage.

DAVID R. MERRILL. 35